

# UNITED STATES PATENT OFFICE.

MAX NIRDLINGER, OF PHILADELPHIA, PENNSYLVANIA, ASSIGNOR TO THE FUEL PATENTS COMPANY, OF NEW JERSEY.

## ARTIFICIAL FUEL.

SPECIFICATION forming part of Letters Patent No. 533,486, dated February 5, 1895.

Application filed March 23, 1892. Serial No. 426,147. (No specimens.)

*To all whom it may concern:*

Be it known that I, MAX NIRDLINGER, a citizen of the United States, residing at Philadelphia, in the county of Philadelphia and State 5 of Pennsylvania, have invented certain new and useful Improvements in Artificial Fuel, of which the following is a specification.

This invention relates to an improved composition of materials for a fuel, the object being to provide a fuel of coal dust, slack or culm, which shall be of little cost, and shall be capable of compression into blocks or cakes that will maintain their form and desired consistency under all ordinary conditions.

15 Heretofore much difficulty has been experienced in producing a fuel containing the slack or culm of coal which will meet all the requirements of a marketable article. In some cases the fuels after they have been 20 manufactured into the form of blocks or cakes disintegrate rapidly either because of the absorption of moisture or from the contraction and expansion due to variations in temperature. With others it is found that as soon as 25 the fuel is introduced into the fire a disintegration there immediately results from the heating or evaporating of the binding ingredients.

I have found that a superior fuel can be 30 provided by combining in suitable proportions the culms of the two distinct species of coal known as the bituminous and the anthracite, and also that a very efficient binding material can be produced by using pitch, together with a small amount of the tar obtained 35 from that pitch during the process of distillation. I manufacture it as follows: Eighteen hundred pounds of culm, slack, dust or screenings of anthracite coal are placed in a mixing 40 machine and thoroughly mingled with one hundred pounds of the culm, slack or screenings of bituminous coal; and they are heated to a comparatively high temperature (100° Fahrenheit) and are thoroughly freed from moisture. Then the binding material is provided 45 as follows: About ninety pounds of hard coal tar pitch are heated, to which are added about ten pounds of coal tar. The tar or oil product is obtained in the same process of distillation or manufacture which produces the 50 aforesaid hard pitch. It is practically im-

possible to stop the process of distillation or manufacture at the point where there is a pitch material suitable for my purposes. Hence I find it necessary to take the pitch 55 after its manufacture and again add thereto a small amount of the tar previously taken therefrom in order to produce a compound which will be capable of being made sufficiently fluid to be mixed with the other ingredients and yet shall after the fuel is manufactured be sufficiently hard at all ordinary temperatures to meet the requirements.

Heretofore there has not been, so far as I know, any discovery or utilization of the principle which I follow, namely, this, that there is a certain advantageous coaction between the hard pitch and its companion tarry or more viscid product. I am aware of the fact that in numerous ways pitches, tars, resins, &c., have been commingled; but I have found that if a vegetable product be combined with the mineral, or vice versa, the efficiency of the binder is practically destroyed. In other words, I have succeeded in producing a binder 75 which at all ordinary temperatures is thoroughly solid, but the proportions are such that at the time of manufacture it is softened only to the point where a thorough commingling of it with the solid particles is attainable.

After the two species of the coal, culm or slack have been thoroughly commingled, heated and dried, and after the above-described hydrocarbon and other ingredients 85 have been properly mixed, they are placed together (in the proportions of nineteen hundred pounds of the mixed culms to one hundred pounds of the hydrocarbon) in a mixing machine, where they are thoroughly agitated 90 and mixed together and are heated to the temperature of 175° Fahrenheit. In this way a homogeneous mass is produced which contains the above ingredients uniformly distributed throughout. After the mixing is 95 thoroughly effected, the material is passed to a machine whereby it is compressed into small, hard blocks or cakes of about the size of large hen-eggs, which upon becoming cool and dry are ready for the market.

100 I have found that the mixture of the anthracite and bituminous coal in about the

proportions named is a matter of great advantage. The particles of the anthracite coal are so hard and have faces and edges which are so smooth and sharp that it is difficult to bind them together by any of the ordinary compounds to such an extent that they will permanently maintain the forms into which they may be compressed. Especially is it true that as soon as the high heat of a fire is applied disintegration occurs, and it is impossible to get the desired "coking" effect; but the bituminous coal is charged with hydrocarbon elements to such an extent that as soon as heat is applied the fusion of the particles of the coal acts to assist in binding together the particles of the anthracite coal. In short, the bituminous coal may be regarded as a material intermediate between the pitch and the anthracite and adapted to assist not only in binding the particles of the fuel together but also to assist, under a high heat, in securing a "coking" effect.

Of course I am aware that many fuel compositions have heretofore been patented, and that it has been proposed to use in various ways the ingredients which I have above set forth; but I am familiar with all of the fuels that have been patented and also with many that it has been attempted to manufacture, and I do not believe the composition which is

above described and produced in the way set forth has ever been provided for.

What I claim is—

1. The herein described improvement in the art of manufacturing artificial fuel, the same consisting in mixing and thoroughly commingling anthracite and bituminous coal, heating the mass whereby all the moisture is expelled; then melting hard coal tar pitch and mixing with it while in a heated condition, coal tar obtained in the manufacture of pitch; then mixing and commingling the two masses while in a heated condition, subjecting the resulting mixture to pressure and forming it into small blocks or balls, substantially as set forth.

2. The herein described carbonaceous fuel it comprising ninety pounds of hard coal tar pitch, ten pounds of coal tar obtained in the manufacture of said pitch, eighteen hundred pounds of the slack of anthracite coal, and one hundred pounds of the slack of bituminous coal, substantially as set forth.

In testimony whereof I affix my signature in presence of two witnesses.

MAX NIRDLINGER.

Witnesses:

C. M. HOOPER,

W. G. MARSON.